

## UNITED STATES PATENT OFFICE

2,282,810

## METHOD FOR STABILIZING OILS

Sidney Musher, New York, N. Y., assignor to  
Musher Foundation Incorporated, New York,  
N. Y., a corporation of New York

No Drawing. Application July 31, 1940,  
Serial No. 348,823

10 Claims. (Cl. 260—398.5)

The present invention relates to the stabilization of glyceride oils and particularly to the stabilization against oxidative deterioration of those glyceride oils which contain a large proportion of unsaturated glycerides.

It has been found that these oils are particularly oxidizable and that this deterioration is increased wherever the oils are subjected to high temperature deodorization during the refining process.

It has now been found that when such glyceride oils are heated to relatively high temperatures with combinations of water soluble carbohydrates and particularly sugars such as dextrose and sucrose on the one hand together with an aromatic compound, preferably at least di-substituted with amino or hydroxy groups on the other hand, instead of losing stability and becoming more subject to deterioration, the oils will become very stable and highly resistant to oxidative deterioration and rancidity.

The sugars and the aromatic compounds are used preferably in equal proportions. They may also be employed in relative proportions varying from about 1 part of the former and 10 parts of the latter to 10 parts of the former and 1 part of the latter, and the combinations are dispersed in the glyceride oil which is then heated or they may be added to the oil during high heat treatment to develop marked antioxygenic effectiveness.

These sugars and aromatic compounds may be added separately to the oil to be stabilized or may first be mixed in combination and then added to the oil but in either case they are thoroughly dispersed in the oil and held dispersed in the oil while the oil is at an elevated temperature in excess of 250° F. and preferably at over 400° F.

The preferred aromatic compounds which are combined with the sugars have desirably a poly-substituted benzene ring excluding such compounds as phenol or aniline. These compounds are the dihydroxy benzenes, the di-amino benzenes, the aminohydroxy benzenes and less preferably similar compounds in which the other substituents in addition to the amino or hydroxy group are the alkyl or aryl group such as aryl phenol or an alkyl aniline or even a second nuclear chain such as, for example, as in the case of an alpha or beta naphthol or an alpha or beta naphthylamine or aminonaphthols, or diamino or dihydroxy naphthalenes.

The preferred aromatic hydroxy compound to use in accordance with this invention is hydro-

quinone. Other useful di- and tri-hydroxy compounds, the hydroxy groups of which may have been etherized, include guaiacol, gum guaiac, phloroglucinol, resorcinol, pyrogallol, pyrocatechol, tri-butylcatechol, vanillin, thymol, and similar compounds.

Still other less preferable useful compounds are included in the general group having the formula

10



15 where  $x$  is at least one OH and preferably includes two OH groups or even alkoxy-groups and may less preferably include  $\text{NH}_2$  or  $\text{COOH}$  or  $\text{CHO}$  or  $\text{CO}$  or alkyl chains including the same; where  $n$  is at least 2; and where  $y$  is hydrogen, 20 aryl, alkoxy, aralkyl, alpharyl, amino, sulfo, aldo, keto or alkyl chains or groups including the same.

As examples of the less preferred compounds included in the classification given above are di-phenylamine, alphanaphthylamine, phenylbeta-naphthylamine, eugenol, gallic acid and gallo-tannin.

Among the other compounds which may also be utilized are ethyl, propyl, butyl, amyl, hexyl, 30 or octyl phenols, anilines, naphthols, hydroquinones, pyrogallols or the methoxy, ethoxy, butoxy ethers, di-hydroxy or di-amino or hydroxy amino naphthalenes, which alkyl groups may or may not be substituted by aryl groups such as 35 phenyl or toluyl such as ethyl, butyl, amyl, hexyl, or octyl. Less preferably it is possible to utilize aryl substituted phenols, anilines, naphthols, naphthylamines, hydroquinones, aminophenols, cresols or xylenols.

40 Among the other compounds that may be specifically employed are polyhydroxybenzenes in which one of the hydroxy groups may be etherified such as hydroxyhydroquinone, 1:2:4 tri-hydroxy benzene, 1:2-di-methyl-3:6-di-hydroxy 45 benzene, 1:2-di-methyl-4:5-di-hydroxy benzene, 1:3-di-ethyl-2:5-di-hydroxy benzene, ethyl pyrogallol, methoxy hydroquinone, pyrogallol-1-methyl ether, ethoxy catechol; or naphthols such as 1:2-di-hydroxy naphthalene, 1:4-di-hydroxy 50 naphthalene; or poly aminobenzenes or aminophenols or aminonaphthols such as di- or triamino benzenes, 1:5 dihydroxy naphthalene, para phenylene di-amine, ortho-aminophenol, para-aminophenol, dimethyl para-aminophenol, di-butyl aminophenol, di-ethyl aminocresol, phenyl-

55

aminophenol, benzyl aminophenol, 2 amino-5-hydroxy toluene, benzyl-p-aminophenol, dibenzyl-p-amino phenol, 2:4 diamino diphenylamine, p,p-diamino-diphenyl amine, phenyl alpha naphthylamine, alkyl alpha naphthylamine; or less preferably other substituted benzenes such as carvacrol, tribromo or trichloro phenols, etc., or other compounds such as furfural or p-hydroxy phenyl morpholine.

The preferred combination of sugar and aromatic compound is a mixture of dextrose and hydroquinone, preferably in equal proportions by weight.

The sugars that are utilized in accordance with the present invention include particularly the monosaccharides such as dextrose and less preferably the di, tri or polysaccharides such as sucrose, maltose, lactose and still less preferably dextrin or solubilized and/or gelatinized starch.

Other sugars that may be utilized for combination with the hydroxybenzenes include raw or refined cane or beet sugar, cane or beet sugar molasses, invert sugar or molasses, corn sugar molasses, carbohydrate alcohols, etc.

The combination is added in an amount of less than 5% and desirably less than 1%. As little as 0.005% to 0.1% will give highly desirable stabilizing results when the glyceride oils are treated in accordance with this invention.

After dispersing the combination of sugar and aromatic compound, such as the combination of dextrose and hydroquinone in the oil, the oil is heated to an elevated temperature, desirably in excess of 250° F. and preferably to between 325° F. and 450° F. for at least 15 to 30 seconds.

It has been found that merely melting a glyceride fat or oil, particularly where the glyceride is solid at room temperature, is not sufficient to give the desired effect and it is necessary to utilize an elevated temperature substantially above the melting point of the glyceride if it normally be solid at room temperature.

During the heating period, the sugar residue may become burnt or charred and, where desired, the burnt residue may be removed as by filtration or centrifuging from the body of the oil, as the stabilization of the oil will already have been effected.

This charring apparently enhances the action of the combination on the oil and it has been found particularly desirable for the heating to be sufficiently high so as to produce charring in order to obtain the fully desirable results of the present invention.

The oil which has been heated with the combination will normally be darker as the result of the elevated temperature treatment and the stabilization will have been effected even though the charred residue be removed from the oil as by filtration or centrifuging. It, however, has been found that the original light color of the oil may be restored by a bleaching process as, for example, with fuller's earth or other decolorizing materials and still retaining a substantial enhancement in the stability of the oil.

The results of the present invention are particularly surprising since antioxidants are recognized as losing at least a portion of, and in most cases a major portion of their effectiveness when heated to elevated temperatures such as to 400° F. or more.

#### Examples I

Bleached refined lard was treated by adding thereto and mixing therein combinations of

sugars and aromatic compounds. The lard containing the combination was then heated to 400° F. for 5 minutes, allowed to cool, and filtered to remove the charred sugar solids. The lard was thereupon tested by bubbling air through a 20 cc. sample of the lard at 125° F. until rancidly as determined organoleptically and by peroxide values was observed. The following results were obtained.

|                                                 | Unheated | After heating to 400° F. for 5 minutes |
|-------------------------------------------------|----------|----------------------------------------|
| 15 Control refined bleached lard (no additions) | Hours 4  | Hours 3                                |
| Lard plus 0.1% dextrose alone                   | 4        | 3½                                     |
| Lard containing 0.1% dextrose plus:             |          |                                        |
| 0.01% hydroquinone                              | 43       | 153                                    |
| 0.005% alphanaphthol                            | 12       | 38                                     |
| 0.01% phenylbetanaphthylamine                   | 13       | 31                                     |

Each of the above materials used with dextrose, when heated in the lard without dextrose results generally in a decrease in stability of the lard.

It is not possible to merely heat the various combinations such as the sugar-hydroquinone combination alone and then add such heated combination to an oil as other antioxidants may be added without further heating and obtain the enhanced stability effect. In order to obtain the interaction it is necessary for the heating to be conducted after dispersal of the combinations in the oil.

The glyceride may, where desired, be bleached or otherwise refined after treatment at the elevated temperature with the combination and a distinct enhancement of the antioxygenic effect will be obtained, such enhancement being far in excess of normal expectation.

It is not desirable for the heating to be conducted in a small body of the oil and that oil used as a base for addition to a large body of oil. The most desirable method is for the combination to be dispersed in the entire body of material to be stabilized, followed by subjecting the oil to a high heat in order to produce the desired interaction or result.

#### Examples II

50 Hydroquinone and sugar were used in lard and tested as above

Rancid after hours

Lard containing 0.005% hydroquinone alone without heating

14

55 Lard containing 0.005% hydroquinone and 0.005% dextrose without heating

14

Lard containing 0.005% hydroquinone and 0.005% dextrose which hydroquinone-dextrose mixture had first been heated without presence of the lard to 400° F., cooled, and then added to the lard with no further heating

10

60 Lard containing 0.005% hydroquinone and 0.005% dextrose which hydroquinone-dextrose mixture had first been heated with 20% of the lard to 400° F., cooled and then added to the remainder of the lard without further heating

17

65 Lard containing 0.005% hydroquinone and 0.005% dextrose heated in the lard to 400° F., cooled, and tested

73

Apparently a chemical reaction occurs between the components of the combination and the oil at the elevated temperature whereby the stabilization is effected, as this reaction does not appear

to be related to ordinary negative oxidation catalysis by means of which antioxidants normally exercise activity.

The higher the temperature to which the oil containing the combination of, for example, hydroquinone and dextrose is subjected, the greater the stabilizing action although the sharpest increase in stabilization is between about 325° F. and 450° F.

The heat treatment need not be prolonged, the enhanced antioxygenic effect being obtained in relatively short periods particularly where the higher temperatures are employed. Normally, the oil containing the combination may merely be heated to the desired temperature and allowed to cool, being held at the high temperature for a period of 10 minutes or more.

The heat treatment will usually be carried out at atmospheric pressure but the use of super or sub-atmospheric pressures may also be employed with satisfactory results.

This process may be utilized in the treatment and stabilization of a wide variety of refined or crude glyceride oils such as the vegetable oils and fats including cottonseed oil, corn oil, peanut oil, linseed oil, soya bean oil, olive oil, etc., the animal oils and fats including lard, tallow, oleo oil, cod liver oil, halibut liver oil, mackerel oil, menhaden oil, herring oil, shark liver oil, butter, etc., the glyceride soap oils and the sulfonated oils.

Not only is the oil stabilized, but components of the oils are also stabilized. For example, the vitamin A content of fish liver and other oils, the carotene content of butter fat and similar substances associated with the oils which may be destroyed or reduced by oxidation are highly stabilized by this treatment.

This invention is, however, particularly beneficial in the treatment of those glycerides which contain large proportions of unsaturated fatty acids, as the combination appears to react more completely with these unsaturated oils at the elevated temperatures.

The sugar, preferably dextrose, is utilized desirably in crystalline and anhydrous form in order to obtain the most enhanced antioxygenic effect.

Although the aromatic compounds and preferably the di-substituted benzene may already have some antioxygenic effect when added to the glyceride oils and without the heat treatment, nevertheless such antioxidant power is very greatly increased and enhanced by heating the combination in the oil to over 250° F. and preferably to 325° F. to 450° F.

The stability of the treated oils will often be enhanced from 50% to 500% or more by the heat treatment in the presence of these combinations as compared to the stability which would be obtained by the addition of the combinations without the heat treatment described in this invention.

The most important features of the present invention reside in the fact that the added materials are not normally present in the oil to be stabilized and upon addition are thoroughly dispersed in such oil. The heat treatment is carried out for a sufficient length of time to increase the stability by usually not less than 50% over the stability of the unheated oil.

While the combination is dispersed in the oil at the elevated temperature of, say 400° F., superheated steam may, where desired, be continuously injected into the oil over a period as long

as 4 to 6 hours and the objectionable flavors and odors originally present in the oil may be removed therefrom while the combination is exerting its enhanced antioxygenic effect.

5 It has been found particularly desirable for a small amount of the combination to be added to high fat containing animal products, heating at atmospheric or elevated pressures to temperatures of about 250° F. so that the glyceride oil or fat 10 contained therein is released from the meat or fish animal product and a highly stabilized animal glyceride is obtained.

For example, to a kettle of hog fat containing 70% total glycerides may be added 0.02% of a combination of gum guaiac and dextrose against the weight of the hog fat and the combination placed in a steam kettle with steam being injected into the kettle to produce about 45 pounds pressure. After a 4 to 6 hour treatment, the pressure may be released and the rendered lard removed. The stability of the lard obtained in this manner will be much greater than if the combination had merely been added to the lard after rendering.

15 For example, when a small amount of a combination of gum guaiac and dextrose is added to hog fat and the hog fat containing the combination is then rendered at a temperature of 275° F. for 4 hours, the rendered lard removed from the rendering kettle has a far greater stability 20 than where a proportionate amount of the combination is added to the lard after rendering and the improvement in stability is even greater than where the combination is added to the lard 25 after rendering and the lard containing the combination is then heated to 275° F. for 4 hours. Apparently a further interaction takes place by adding the combination to the rendering kettle 30 where the rendering is conducted at over 250° F. resulting in a most highly stabilized oil.

35 In a similar manner, a small amount of the combination may be added to the rendering kettle in the rendering of other meat and fish oils and fats including tallow, menhaden oil, herring oil, etc., or to the cooking kettles in the manufacture 40 of fish meals, particularly high glyceride containing fish meals, and where the temperature is at least about 250° F., the desired interaction 45 will result producing enhanced stabilization.

50 Where the glyceride oils are heated over long periods to temperatures over 250° F. and desirably to temperatures over 300° F., small amounts of the combination may be added to the oils at regular intervals of 5 to 20 hours followed by 55 filtration to remove the insoluble portion before adding a fresh amount of the combination. In this manner, the glycerides will be held in highly stabilized and non-rancid condition over very long periods.

60 In addition to treating the glyceride oils and fats with these combinations, the essential oils and particularly the oxidizable unsaturated essential and perfume oils such as lemon oil and orange oil may similarly be treated with the combinations followed by an elevated temperature treatment to enhance the antioxygenic effect.

65 The combinations also exert an enhanced antioxygenic effect when added in small proportions to the substantially non-volatile, high molecular weight, hydrocarbon oils and particularly the lubricating oils followed by temperature treatments of over 250° F. and preferably between 70 350° F. and 500° F.

75 In carrying out the above described high temperature treatment, it is important that the solids

of the combinations be uniformly dispersed or distributed throughout the body of the oil in substantially fine particles and that the heating be carried out with substantial exclusion of the atmosphere or without contact with air.

It is moreover desirable for the combination to be maintained in dispersed condition during the heat treatment and so that it will not tend to settle or conglomerate or be present in the form of large lumps or particles since in the latter case the fully desirable results of the present invention are not obtained.

It is desirable that the oil after treatment in accordance with the present invention will not be materially changed in its odor or flavor. The oil will, however, have a darker color which may be removed by subjecting it to a bleaching operation.

It has also been found that desirable results are obtained where the combinations are mixed with the oil or fibrous materials containing the glyceride oil and then the oil is heated to a temperature of, say from 250° F. to 500° F. under a reduced pressure, such as under a gas pressure less than 1 pound per square inch, to cause distillation of part or all of the glyceride oil composition and it has been observed that such distilled fraction is highly stable and is also free of the combination which has served as the stabilizing agent at the elevated temperature of distillation.

After treatment of the glyceride oil with the combination at the elevated temperature, the unsaponifiable fraction may be removed as by alcoholic extraction and said unsaponifiable fraction utilized for addition to other oxidizable oils to protect them against oxidative deterioration.

Combinations of sugars and hydroxylamine may also be employed for addition to the oils followed by the heat treatment to over 250° F.

The present application is a continuation in part of application Serial No. 247,631 filed December 24, 1938, and through said application was copending with application Serial No. 249,166 filed January 3, 1939, now Patent No. 2,198,210; application Serial No. 292,613 filed August 30, 1939, now Patent No. 2,198,208; application Serial No. 260,898 filed March 10, 1939, now Patent No. 2,198,211; and application Serial No. 304,945, filed November 17, 1939, now Patent No. 2,216,711. The present application is particularly directed to the use of a poly hydroxy aromatic compound and a water soluble carbohydrate, particularly hydroquinone and sugar, in the treatment of glyceride oils when accompanied by a heat treatment to stabilize such oils against oxidative deterioration.

Having described my invention, what I claim is:

1. A process of stabilizing oils subject to oxidative deterioration, whereby they become less subject to such deterioration, which comprises adding thereto and dispersing therein a small amount of a water soluble carbohydrate and a small amount of a compound having the general formula



where  $x$  is a radical selected from the group consisting of OH, alkoxy, NH<sub>2</sub>, COOH, CHO, CO and alkyl chains including the same, where  $n$  is at least 2 and where  $y$  is a radical selected from the

group consisting of hydrogen, aryl, alkoxy, aralkyl, alpharyl, amino, sulpho, aldo, keto and alkyl chains including the same, and heating to in excess of 250° F.

5. A process of stabilizing oils subject to oxidative deterioration whereby they become less subject to such deterioration, which comprises adding thereto and dispersing therein a small amount of a combination of a water soluble carbohydrate and a polyhydroxy aromatic compound, and heating to in excess of 250° F. while the oil is under sub-atmospheric pressure.

3. A process of stabilizing glyceride oils subject to oxidative deterioration whereby they become less subject to such deterioration, which comprises adding thereto and dispersing therein a small amount of a combination of a sugar and a polyhydroxy benzene, and heating to in excess of 250° F.

20. 4. A process of stabilizing glyceride oils subject to oxidative deterioration whereby they become less subject to such deterioration, which comprises adding thereto and dispersing therein a small amount of a combination of a sugar and hydroquinone, and heating to in excess of 250° F.

25. 5. A process of stabilizing oils subject to oxidative deterioration, whereby they become less subject to such deterioration, which comprises adding thereto and dispersing therein a small amount of a combination of a water soluble carbohydrate and an aminohydroxy aromatic compound, and heating to in excess of 250° F.

30. 6. A process of stabilizing oils subject to oxidative deterioration, whereby they become less subject to such deterioration, which comprises adding thereto and dispersing therein a small amount of a combination of a water soluble carbohydrate and an aminohydroxy benzene, and heating to in excess of 250° F.

35. 7. An oil normally subject to oxidative deterioration carrying the reaction product of a water soluble carbohydrate and an aromatic compound in the oil, said aromatic compound having the general formula



where  $x$  is a radical selected from the group consisting of OH, alkoxy, NH<sub>2</sub>, COOH, CHO, CO and alkyl chains including the same, where  $n$  is at least 2 and where  $y$  is a radical selected from the group consisting of hydrogen, aryl, alkoxy, aralkyl, alpharyl, amino, sulpho, aldo, keto and alkyl chains including the same, said reaction product having been formed by heating the combination in the oil to a temperature in excess of 250° F. whereby an enhanced antioxygenic effect is obtained.

40. 8. A glyceride oil having a high proportion of unsaturated glycerides, said oil being normally subject to oxidative deterioration, said oil carrying the reaction product of a combination of a sugar and a polyhydroxy benzene, said reaction product having been formed by heating the combination in the oil to a temperature in excess of 250° F. whereby an enhanced antioxygenic effect is obtained.

45. 9. A glyceride oil normally subject to oxidative deterioration carrying the reaction product of a combination of a water soluble carbohydrate and an aminohydroxy benzene, said reaction product having been formed by heating the combination

in the oil to a temperature in excess of 250° F. whereby an enhanced antioxygenic effect is obtained.

10. A process of stabilizing glyceride oils subject to oxidative deterioration, whereby they become less subject to such deterioration, which comprises adding thereto and dispersing therein a small amount of a water soluble carbohydrate and a small amount of a compound having the general formula

where  $x$  is a radical selected from the group consisting of OH, alkoxy, NH<sub>2</sub>, COOH, CHO, CO and alkyl chains including the same, where  $n$  is at least 2 and where  $y$  is a radical selected from the group consisting of hydrogen, aryl, alkoxy, aralkyl, alpharyl, amino, sulpho, aldo, keto and alkyl chains including the same, heating to in excess of 250° F., and then removing the unsaponifiable fraction therefrom.

10

SIDNEY MUSHER.

